

## UNITED STATES PATENT OFFICE.

FRANCIS C. TÉLEN, OF PENNS GROVE, NEW JERSEY, ASSIGNOR TO E. I. DU PONT DE NEMOURS & COMPANY, OF WILMINGTON, DELAWARE, A CORPORATION OF DELAWARE.

## PROCESS OF MORDANTING AND DYEING WOOL.

No Drawing.

Application filed July 1, 1921. Serial No. 481,982.

*To all whom it may concern:*

Be it known that I, FRANCIS C. TÉLEN, a citizen of the United States, and a resident of Penns Grove, in the county of Salem and

5 State of New Jersey, have invented a certain new and useful Process of Mordanting and Dyeing Wool, of which the following is a specification.

This invention relates to the mordanting 10 of wool with chromium compounds and the dyeing of the wool in the presence of the mordanting liquor. One of the essential features of my invention is the reduction of the chromium compound, for example, 15 sodium bichromate, with lactic acid in the absence of stronger acids such as sulphuric. Another important feature of my invention consists in adding the dye directly to the mordanting bath.

20 As is well known, mordant dyestuffs, including the ortho-oxy-azo colors, form colored lakes with the metals. This fact is made use of in the application of these dyes, the most valuable and most extensively 25 used lakes of these colors being those of chromium. These chromium lakes are produced on the fibre either by mordanting the material with chromium salts and then dyeing with the particular color, or by using the 30 so-called chromate, mono-chrome, meta-chrome, or after-chrome processes. When these colors are dyed in metal machines, especially machines constructed of iron, the formation of the valuable chromium lake is 35 interfered with by the presence of the iron, and in consequence, the dyeings are rendered valueless. It has therefore been customary to carry out the mordanting and dyeing operations in vessels made of wood or having a 40 non-metallic inner surface.

One object of my invention is to provide a process of chrome-mordanting and dyeing which will permit the use of iron, or other metallic, vessels.

45 Another object of my invention is to improve on methods of applying chrome colors, and especially chromable azo dyestuffs, whereby a great saving in time may be effected.

50 I have discovered that lactic acid combines to an eminently satisfactory degree the

two properties of being a sufficiently strong reducing agent to reduce bichromates without the assistance of other acids, and sufficiently weak to have no appreciable action 55 on iron. It is possible that the avoidance of injurious results from the presence of iron may be due to some positive, instead of to a negative, behavior of the lactic acid, but that the excellent results obtained are due to the 60 inability of the lactic acid to attack metals such as iron seems most probable.

I have discovered, furthermore, that, irrespective of the type of vessel used, a great economy in time may be effected by using 65 lactic acid as the reducing agent for the bichromate, and, after a short preliminary treatment of the wool in the mordanting bath, adding the dyestuff directly to said bath, the last step of the operation being an 70 after-chroming treatment.

My new process as carried out in an iron vessel may be illustrated by the following example:

100 lbs. of wool are boiled with from 75 about 1,000 to 1500 pounds of water containing  $2\frac{1}{2}$  lbs. of sodium bichromate (hydrate) and 5 lbs. of lactic acid for 30 minutes. To this solution is added the required amount of dyestuff, for example, 6 lbs. of 80 2,2'-dihydroxy-4-sulfo-1,1'-azonaphthalene previously dissolved in hot water. The dyeing is continued for one hour with the addition of organic or mineral acids (for example, sulphuric acid) to exhaust the 85 color. The color is then after-chromed in the same, or in a fresh, bath with 2 lbs. sodium bichromate, one pound of sulphur acid and 4 lbs. of lactic acid for 30 minutes. Where a fresh bath is used the bichromate, 90 sulphuric acid and lactic acid are dissolved in from 1000 to 1500 lbs. of water, depending upon the capacity of the dyeing machine used. The above steps of mordanting and dyeing are preferably carried out with boiling solutions; if desired, however, the solutions may be maintained at a temperature between about 90 and 100° C. 95

The above procedure represents a combined method of dyeing and mordanting, 100 and depends for its utility, on the partial reduction of bichromate or other chromium

salts by lactic acid and its salts. The reduction takes place on the fibre so that enough chromic oxide is formed on the fibre to negative the bad effects of the presence of 5 iron or other material entering the dye bath from the dyeing machine, thus insuring a pure shade. It also insures the same fullness and depth and the same fastness that would be obtained from the same amount of color 10 by any other method of chroming.

It will be readily appreciated by those versed in the art that this method marks a distinct improvement, in that it effects a great economy in time. By the older 15 methods it is found necessary to mordant the goods for at least 1½ hours in order to effect the complete reduction of the bichromate, and then the dyeing must be carried out in fresh liquor. In my process, this time is 20 cut down, because after the reduction has proceeded only a little way, the dyeing can be carried out in the same liquor. The final after-chroming, as described in the example, 25 is given only to insure the greatest possible fastness.

It will be understood that the process of using lactic acid with the exclusion of other stronger acids to overcome the injurious action of iron or iron salts is of general application in the chrome-mordanting of wool, and that the process, as regards the series of steps, may be practiced with various dyes other than the azonaphthalene derivative above-mentioned. The conditions of operation given in the specific example may also be varied considerably as will be evident to one skilled in the art.

I claim:

1. A process permitting the mordanting 40 of wool with a bichromate solution in a vessel provided with an inner metallic surface, composed, at least in part, of a metal whose salts are capable of reacting with mordant dyestuffs to form colored lakes which comprises treating the wool with a hot solution 45 containing a bichromate and lactic acid but free from an acid substantially stronger than lactic acid, said solution during at least part of said treatment being in contact with part of said metallic surface.

2. The process which comprises treating 55 wool with a boiling solution containing a bichromate and lactic acid but free from an acid substantially stronger than lactic acid, said solution during at least part of said treatment being in contact with a metal whose salts are capable of reacting with mordant dyestuffs to form colored lakes.

3. The process which comprises treating 60 wool with a hot solution containing a bichromate and lactic acid but free from an acid substantially stronger than lactic acid, said solution during at least part of said treatment being in contact with metallic iron.

4. The process which comprises subjecting wool in an iron vessel to the action of a solution containing an alkali-metal bichromate and lactic acid but free from an acid capable of dissolving part of the iron, 70 said solution being maintained at a temperature of from about 90 to 100° C.

5. The process which comprises subjecting wool in an iron vessel to the action of a boiling solution containing sodium bichromate and an acid component composed 75 of lactic acid.

6. The process of dyeing wool which comprises treating that wool for about half an hour with a solution at a temperature 80 of from about 90 to 100° C. containing a bichromate and lactic acid, then adding to the resulting mixture a solution of a mordant dyestuff, and heating the bath at a temperature of from about 90 to 100° C. 85 with the addition of an acid to exhaust the color.

7. The process of dyeing wool which comprises treating the wool for about half an hour with a solution at a temperature 90 of from about 90 to 100° C. containing sodium bichromate and lactic acid, then adding to the mixture a water solution of an ortho-hydroxy-azo-dyestuff, maintaining the resulting solution in the presence of said 95 wool at a temperature of from about 90 to 100° C. with the addition of an acid to exhaust the color in the dye bath, and after-chroming the dyed wool with a bichromate 100 solution containing sulphuric and lactic acids.

8. The process of dyeing wool which comprises treating the wool in a vessel having an inner surface of iron for about half an hour with a solution at a temperature 105 of from about 90 to 100° C. containing a bichromate and lactic acid, then adding to the resulting mixture a solution of a mordant dyestuff, and heating the bath at a temperature of from about 90 to 100° C. 110 with the addition of an acid to exhaust the color.

9. The process of dyeing wool which comprises treating the wool in a vessel having an inner surface of iron for about half 115 an hour with a solution at a temperature of from about 90 to 100° C. containing a sodium bichromate and lactic acid, then adding to the mixture a water solution of an ortho-hydroxy-azo-dyestuff, maintaining the 120 resulting solution in the presence of said wool at a temperature of from about 90 to 100° C. with the addition of an acid to exhaust the color in the dye bath, and after-chroming the dyed wool with a bichromate 125 solution containing sulphuric and lactic acids.

10. The process of dyeing wool which comprises maintaining 100 parts of wool in contact for about half an hour with a boil- 130

ing solution containing about  $2\frac{1}{2}$  parts of sodium bichromate and about 5 parts of lactic acid, then adding a water solution containing about 6 parts of 2,2'-dihydroxy-

and then after-chroming the dyed wool with about 2 parts of sodium bichromate, about 1 part of sulfuric acid and about 4 parts of 10 lactic acid.

- 5 4-sulfo-1,1'-azonaphthalene, boiling the resulting solution for about an hour with the addition of an acid to exhaust the color,

In testimony whereof I affix my signature.

FRANCIS C. TELEN.